

## UNITED STATES PATENT OFFICE

2,370,332

## TREATMENT OF CELLULOSE MIXED ESTERS

Howard A. Tanner, Rochester, N. Y., assignor to  
Eastman Kodak Company, Rochester, N. Y.,  
a corporation of New Jersey

No Drawing. Application March 14, 1941,  
Serial No. 383,369

13 Claims. (Cl. 106—171)

This invention relates to the manufacture of sheeting and photographic film base and more particularly to a method of treating cellulose mixed organic acid esters employed as the base of the sheeting and film base whereby the adhesion of the sheet or film is reduced, and whereby no viscosity change is produced in the solution from which the sheet or film base is coated.

Photographic films and similar films and thin sheeting commonly employed for wrapping materials are usually prepared from cellulose esters by coating a solution of the cellulose ester onto a smooth coating surface and then stripping off the film or sheet after the solvents have been partially evaporated. In the case of single esters no great difficulty has been experienced in stripping the formed film or sheet from the coating surface. However, when cellulose mixed organic acid esters were coated from solvent solutions and in particular from chlorinated solvents in accordance with the "gel dope" process described in Fordyce application Serial No. 245,023, filed December 10, 1938, now U. S. Patent No. 2,319,055, issued May 11, 1943, appreciable difficulty was experienced from time to time with the adhesion of the sheet or film to the coating surface. In some instances such adhesion caused particles of the film to be pulled away or the film to be torn with the result that the product was unusable.

Various attempts were made to overcome this adhesion of the mixed ester sheets. It was finally found that if the mixed ester were treated with an aqueous sodium or potassium soap solution that the adhesive characteristic of the resulting film base or sheet could be controlled. However, if the soap treated mixed ester were made into a coating solution in a chlorinated solvent, the improvement in adhesive control was offset by a persistent drift in solution viscosity. It was found that on standing the solution would gradually turn to a gel. This viscosity change greatly interfered with production of sheets by the above mentioned "gel dope" process. This is a phenomenon which is frequently encountered when alkali metal salts (such as sodium stearate) are present in solutions of cellulose esters in solvents containing chlorinated hydrocarbons. The alkali metal ion evidently initiates or catalyzes a breakdown of the chlorinated solvent liberating acidic materials which cause the ester to decompose. This effect may be prevented by the addition of small amounts of a weakly acidic material such as stearic acid or boric acid to repress the formation of alkali metal ions.

The instant application describes an improved method whereby a soap treatment may be employed to control the adhesiveness of the cellulose mixed ester sheets as well as the viscosity of the coating solution particularly when employing chlorinated solvents.

An object of the present invention is a method of reducing the inherent sticking tendency of films, foils and sheets made of cellulose mixed organic acid esters.

Another object of the invention is a method for reducing the adherence of cellulose mixed ester sheets to sheet forming surfaces.

A further object of the invention is a method of reducing the adherence of cellulose mixed ester sheets and film base without producing a tendency for viscosity increases in the solution from which the sheet or film base is coated.

In accordance with the invention these and other objects are attained by soaking the cellulose mixed organic acid ester in an aqueous sodium or potassium soap solution to thoroughly wet the ester with the soap solution. The soap solution is then drained off and the ester rinsed in distilled water to remove all but a minor per cent of the sodium or potassium soap solution. The washing is carried out sufficiently that no more than 1%, preferably no more than 0.5% of the soap remains in the cellulose ester. Ordinarily at least 0.1% of soap is retained by the cellulose ester after the washing operation. The mixed ester is now washed with artificially hardened water containing one or more soluble salts of metals such as calcium, magnesium, zinc, aluminum and copper thereby changing the residual sodium or potassium soap to the corresponding metal soap which is insoluble and of weaker basicity than soaps of sodium or potassium. The ester is then drained free of the artificially hardened water and thoroughly rinsed with distilled water to remove the soluble sodium or potassium salts. This leaves only minor quantities of insoluble metal soaps in the ester which do not react with chlorinated solvents to increase the solution viscosity or cause it to gel. The ester is then dried and mixed in a solvent to form a cellulose mixed organic acid ester coating solution. The solution may then be coated by the process disclosed in Fordyce et al. application Serial No. 335,336, filed May 15, 1940, now Patent No. 2,295,394, into films and sheeting, if the solvent is a chlorinated solvent of the type described therein, or by the process described in Davidson Patent 2,051,201 if the solvent is acetone or other such non-chlorinated solvent.

I have found that by the instant method a sheet or film of a greatly reduced adherence tendency may be made. The product is of good clarity, has a pleasant smooth feel, and slides easily over itself or other surfaces and will freely strip from the coating surface. When chlorinated solvents are employed there is no viscosity change over long periods of time.

The soap solution is preferably a pure dilute solution of sodium stearate soap or a similar soap such as sodium or potassium palmitate and oleate. The concentration of soap in the soap solution does not appear critical and may be in the range of approximately .05 to 10%. The soaking treatment may vary from fifteen minutes to several hours. Ordinarily the temperature of the soap solution may be that of the room although it may be raised somewhat, if desired. If chlorinated solvents are employed the final washing is generally continued until only 0.1 to 0.2% of insoluble metal soap, based on the weight of the cellulose mixed ester, remains held by the mixed ester.

The following are typical examples of how my invention may be applied in forming thin sheeting or film base but are not to be considered as limitations thereof.

#### Example I

A cellulose acetate butyrate containing 19% acetyl and 27% butyryl was repeatedly washed with distilled water after which the acetate butyrate was covered with distilled water and boiled for several hours. It was then again washed several times after which it was covered with 20 times its weight of distilled water and given a soap treatment. This involved heating the water to about 140°-150° F., and then adding with stirring a quantity of warm (150° F.) 10% soap solution to result in a concentration of .05-.1% sodium stearate in the water. After one hour at 140° F. the soap solution was pumped off and the product again covered with twenty times its weight of distilled water. This was again heated to 140° F., allowed to stand for at least ten minutes, and the water drained from the mixed ester. The ester was then immersed for one hour in about 20 times its weight of distilled water which has been artificially hardened by adding a 0.1% solution of aluminum chloride. This is maintained at a temperature of 140° F. This results in a double decomposition reaction and the residual sodium stearate left in the mixed ester is transformed to insoluble aluminum stearate and the sodium combines with the chloride. The water is then drained off and the mixed ester is washed thoroughly with hot distilled water and dried. The drying operation employed is to centrifuge the mixed ester, until it contains only about three times its weight of water, after which it is placed in a drier and dried at about 180° F. to a moisture content of approximately 0.5%.

For film manufacture, the cellulose acetate butyrate thus treated with the soap solution was dissolved in a solvent mixture consisting of 90% by weight of propylene chloride and 10% methyl alcohol to a solvent ratio of about 6:1. Dibutyl phthalate was added as plasticizer to the extent of 25 parts for 100 parts of cellulose ester. The dope was prepared by mixing thoroughly at a somewhat elevated temperature such as 120°-140° F. and was then filtered. It was found that even after prolonged standing there was no tendency for the solution to increase in viscosity or to gel. When supplied to a film coating machine

such as described in Fordyce et al. application Serial No. 335,336, now U. S. Patent Number 2,295,394, issued Sept. 8, 1942, the film exhibited no tendency to adhere to the coating wheel and was easily stripped therefrom.

#### Example II

A cellulose acetate propionate containing 29% acetyl and 15% propionyl was treated according to the method described in Example I with the exception that a 0.1% copper sulfate solution was employed in place of the aluminum chloride solution in which case the residual sodium stearate is changed to insoluble copper stearate and the sodium removed by washing as sodium sulfate. The treated ester was dissolved in 85% propylene dichloride and 15% methyl alcohol and coated on a clean glass surface. The cured film showed no adhesion to the glass surface and was easily stripped therefrom. Portions of the solution not coated showed no tendency to increase in viscosity or to gel.

#### Example III

A cellulose acetate butyrate containing 31% acetyl and 15% butyryl was treated with the washing and soap treatment described in Example I with the exception that a 0.1% magnesium sulfate solution was employed in place of the aluminum chloride solution in which case the residual sodium stearate is changed to insoluble magnesium sulfate and the sodium removed as sodium sulfate. When thoroughly dried the ester was put in solution in a solvent mixture of 300 parts of propylene chloride and 100 parts of ethylene chloride by mixing the ingredients with stirring at 70° C. The solution was then formed into film support by the process and apparatus described in Fordyce application Serial No. 335,335, now Patent No. 2,295,280. No difficulty was experienced in stripping the formed film from the coating surface. Portions of the solution not coated exhibited no viscosity increase or gelation tendency.

#### Example IV

A cellulose acetate propionate containing 30% acetyl and 14.5% propionyl was treated according to the procedure shown in Example I. This ester was made into a coating solution in 600 parts by weight of a solvent mixture composed of 53% by weight of propylene chloride and 47% by weight of amyl alcohol and 10% triphenyl phosphate based on the weight of the ester. When coated according to the process described in Fordyce application Serial No. 335,335, now U. S. Patent Number 2,295,280, issued September 8, 1942, no appreciable adherence of the film to the coating wheel was noted. The viscosity of this solution did not increase on standing.

A small percentage of the insoluble soap based on the weight of the cellulose mixed organic acid ester remains in the sheet or film when the ester is washed as described above. However, I have found by actual tests that a similar amount of soap added to a cellulose mixed organic acid ester solution after the ester and solvent have been mixed will not produce the same result as is obtained by soaking the ester itself in a soluble soap solution and then treating it to change it to an insoluble less basic soap as described. One noticeable result is the reduction in viscosity of the ester when treated by my process. Although I have not determined the exact physical or chemical theory of my invention I have been able to greatly reduce the adherence of sheets and films

without diminishing other desirable characteristics.

As indicated above, the adhesiveness of the cellulose mixed organic acid ester solution may be controlled by employing the soap treatment without the subsequent hardened water wash, but in this case the solution should be formed into the sheeting soon after it is made up otherwise the solution will exhibit a viscosity increase. Furthermore, if acetone or some other solvent which does not have a gelling action or at least as active a gelling action as do chlorinated solvents the hardened water wash may be omitted and the reduction of the adhesiveness of the sheet by the soap treatment will be obtained.

My invention is applicable to any suitable cellulose mixed organic acid ester such as cellulose acetate propionate, and cellulose acetate butyrate, cellulose propionate butyrate, cellulose acetate propionate butyrate, cellulose acetate stearate, cellulose acetate palmitate, cellulose acetate laurate and the like.

The salts employed to harden the distilled water may be aluminum chloride, stannous chloride, copper sulfate, zinc sulfate and magnesium sulfate. The zinc and tin salts are less desirable since they seem to cause haze in the sheeting.

In the accompanying claims the term "sheeting" is meant to include sheeting such as that employed for wrapping purposes as well as that employed for photographic film base.

While I have found that potassium and sodium soaps are very satisfactory for use in carrying out this invention I may in general employ any water soluble soaps including ammonium soaps.

I claim:

1. The method of preparing a cellulose mixed organic acid ester coating solution which comprises treating the ester forming the base of the solution with an aqueous soap solution selected from the group consisting of sodium and potassium soap solutions, washing the soap from the ester with distilled water until 0.1 to 1% of soap based on the weight of the ester remains, treating the ester with artificially hardened water containing soluble salts of one or more metals selected from the group consisting of calcium, magnesium, zinc, aluminum and copper, washing the ester substantially free from the soluble alkali metal salts, drying the ester and mixing the ester and a plasticizer in a solvent to form a solution.

2. The method of preparing a cellulose acetate butyrate coating solution which comprises treating the ester forming the base of the solution with an aqueous soap solution selected from the group consisting of sodium and potassium soap solutions, washing the soap from the ester with distilled water until 0.1 to 1% of soap based on the weight of the ester remains, treating the ester with artificially hardened water containing soluble salts of one or more metals selected from the group consisting of calcium, magnesium, zinc, aluminum and copper, washing the ester substantially free from the soluble alkali metal salts, drying the ester and mixing the ester and a plasticizer in a solvent to form a solution.

3. The method of preparing a cellulose acetate propionate coating solution which comprises treating the ester forming the base of the solution with an aqueous soap solution selected from the group consisting of sodium and potassium soap solutions, washing the soap from the ester with distilled water until 0.1 to 1% of soap based on the weight of the ester remains, treating the ester with artificially hardened water containing soluble salts of one or more metals selected from the group consisting of calcium, magnesium, zinc, aluminum and copper, washing the ester substantially free from the soluble alkali metal salts, drying the ester and mixing the ester and a plasticizer in a solvent to form a solution.
4. The method of reducing the adhesive properties of a cellulose mixed organic acid ester without increasing its tendency to gain in viscosity when in solution in organic solvents which comprises treating the mixed ester with an aqueous soap solution, and washing the soap from the ester with a solvent of the soap until 0.1 to 0.5% of soap based on the weight of the ester remains.
5. The method of reducing the adhesive properties of a cellulose mixed organic acid ester without increasing its tendency to gain in viscosity when in solution in organic solvents which comprises treating the ester with an aqueous soap solution selected from the group consisting of a sodium soap solution and a potassium soap solution, washing the soap from the ester with distilled water until 0.1 to 1% of soap based on the weight of the ester remains, then treating the ester with artificially hardened water containing soluble salts of one or more metals selected from the group consisting of calcium, magnesium, zinc, aluminum and copper, and washing the ester substantially free from the soluble alkali metal salts.
6. Cellulose mixed organic acid ester sheeting containing 0.1 to 0.2% of an insoluble metal soap therein.
7. Cellulose acetate propionate sheeting containing 0.1-0.2% of an insoluble metal soap therein.
8. Cellulose acetate butyrate sheeting containing 0.1-0.2% of an insoluble metal soap therein.
9. Cellulose mixed organic acid ester sheeting containing 0.1-0.2% of an aluminum soap therein.
10. Cellulose acetate propionate sheeting containing 0.1-0.2% of aluminum soap therein.
11. Cellulose mixed organic acid ester sheeting containing 0.1-0.2% of a magnesium soap therein.
12. Cellulose acetate propionate sheeting containing 0.1-0.2% of a magnesium soap therein.
13. The method of reducing the adhesive properties of a cellulose mixed organic ester without increasing its tendency to gain in viscosity when in solution in organic solvents, which comprises treating the mixed ester with an aqueous soap solution, and washing the soap from the ester with distilled water until 0.1-0.5% of soap, based on the weight of the ester, remains.

HOWARD A. TANNER.